

# United States Patent Office

2,829,974

Patented Apr. 8, 1958

1

2,829,974

## TITANIUM-BASE ALLOYS

Walter L. Finlay and Howard T. Clark, Jr., Beaver, Pa., and John A. Snyder, Wilmington, Del., assignors to Rem-Cru Titanium, Inc., Midland, Pa., a corporation of Pennsylvania

No Drawing. Application October 8, 1952  
Serial No. 313,794

5 Claims. (Cl. 75—175.5)

This invention pertains to titanium-base alloys and more specifically to ternary and quaternary alloys of titanium with two or more of the elements chromium, molybdenum and manganese.

This application is a continuation-in-part of our pending applications Serial No. 134,774, filed December 23, 1949, now abandoned, and Serial No. 268,934, filed January 29, 1952, now Patent 2,787,541.

The low temperature or alpha phase of substantially pure titanium, which is of close-packed hexagonal structure, transforms at a temperature of about 885° C., to the high temperature or beta phase, which is of body-centered cubic structure. The presence of such contaminants or alloying agents as carbon, oxygen and nitrogen, in the proportions in which they are commonly found in commercial titanium, tends to raise the beta transformation temperature, and establishes a relatively narrow zone or field of mixed alpha-beta structure. The presence of certain alloying metals, prominent among which are chromium, manganese and molybdenum, has a quite different effect upon transformation. Increasing amounts of these alloying materials tend to stabilize the beta phase at progressively lower temperatures and establish a mixed alpha-beta field of substantial scope.

It has been found that the alloying with titanium of about 12 atomic percent of two or more of the metals manganese, molybdenum and chromium, can be processed to substantially stabilize the titanium in the beta phase at room temperature. The present invention contemplates a group of alloys in which the beta phase has been thus stabilized. Lesser additions of the elements aforesaid result in alloys of excellent properties having a mixed alpha-beta microstructure, and these are likewise contemplated by the present invention.

While atomic percent has been referred to in the preceding paragraph, the proportions appearing elsewhere in this specification and in the claims are weight percent.

The ternary Ti-Mn-Mo alloys of the invention are typified as to strength and ductility by the test results for various analyses given in Table I below:

TABLE I

The physical properties of ternary Ti-Mn-Mo alloys after a 1-hour vacuum anneal at 700° C.

| Composition, percent (balance titanium) |      | Ti base             | Tensile properties, p. s. i. |         | Percent elong. |
|-----------------------------------------|------|---------------------|------------------------------|---------|----------------|
|                                         |      |                     | Yield                        | Tensile |                |
| 1.0                                     | 1.1  | CP <sup>1</sup>     | 92,100                       | 115,800 | 20             |
| 1.8                                     | 2.0  | CP <sup>1</sup>     | 104,300                      | 133,300 | 16             |
| 3.4                                     | 0.8  | CP <sup>1</sup>     | 128,700                      | 136,100 | 19             |
| 3.9                                     | 20.9 | Iodide <sup>1</sup> | 109,400                      | 126,500 | 16             |
| 8.9                                     | 10.2 | CP                  | 125,900                      | 135,600 | 14             |
| 9.4                                     | 5.2  | Iodide              | 128,100                      | 146,100 | 7              |
| 14.5                                    | 5.6  | do                  | 136,500                      | 143,000 | 14             |

<sup>1</sup> CP refers to titanium of commercial purity obtained by magnesium reduction of titanium tetrachloride according to Kroll U. S. P. 2,205,854, while "Iodide" refers to high purity titanium obtained by the iodide process of Van Arkel U. S. P. 1,671,213.

2

It will be seen from the foregoing results that the Ti-Mn-Mo ternaries within the range of about 1 to 15% manganese and 1 to 25% molybdenum have good strength combined with adequate ductility. These alloys have in general at room temperature a mixed alpha-beta microstructure, conducive to relative ease of fabrication, forging, rolling, etc., as compared to the all-alpha or all-beta alloys, while maintaining comparable strengths at room temperature.

10 Considering now the ternary Ti-Mn-Cr alloys of the invention, Table II below gives test data corresponding to Table I for typical analyses:

15

TABLE II

The physical properties of ternary Ti-Mn-Cr alloys after a 1-hour vacuum anneal at 700° C.

20

| Mn | Cr   | Composition, percent (balance titanium) | Ti base | Tensile properties, p. s. i. |         | Percent elong. |
|----|------|-----------------------------------------|---------|------------------------------|---------|----------------|
|    |      |                                         |         | Yield                        | Tensile |                |
| 25 | 4.8  | 10.3                                    | Iodide  | 133,100                      | 138,000 | 16             |
|    | 15.0 | 5.1                                     | do      | 152,600                      | 156,000 |                |
|    | 15.0 | 5.1                                     | do      | 155,600                      | 156,600 |                |
|    | 9.8  | 10.0                                    | do      | 150,700                      | 157,400 |                |
|    | 3.2  | 1.9                                     | CP      | 111,100                      | 129,900 |                |
|    | 5.5  | 11.6                                    | CP      | 172,700                      | 188,700 |                |

35 For the alloys of this group having good strength combined with sufficient ductility for fabrication purposes, the useful range is about 2 to 12% chromium with about 2 to 15% manganese.

It will be seen by comparison of Tables I and II that the Ti-Mn-Cr ternaries have considerably higher strength than the Ti-Mn-Mo ternaries, and the same is true with respect to the Ti-Cr-Mo ternaries described below. The Ti-Mn-Cr alloys in general have a mixed alpha-beta microstructure at normal or atmospheric temperatures.

40 Table III below gives strength and ductility data on typical Ti-Cr-Mo ternary alloys according to the invention:

TABLE III

The physical properties of ternary Ti-Cr-Mo alloys after a 1-hour vacuum anneal at 700° C.

| Cr | Mo | Composition, percent (balance titanium) | Ti base | Tensile properties, p. s. i. |         | Percent elong. |
|----|----|-----------------------------------------|---------|------------------------------|---------|----------------|
|    |    |                                         |         | Yield                        | Tensile |                |
| 60 | 5  | 10.3                                    | Iodide  | 92,500                       | 126,400 | 19             |
|    | 25 |                                         | do      | 114,600                      | 128,800 |                |

65 The useful range for the ductile alloys is about 3 to 15% chromium with about 1.0 to 25% molybdenum. The alloys having a combined content of about 3.0 to 12% of Cr and Mo have a mixed alpha-beta microstructure, while those above 12% combined Cr and Mo have in general a stable beta structure at normal temperatures.

70 Table IV below gives the physical properties of typical quaternary Ti-Mn-Cr-Mo alloys according to the invention:

**3**  
**TABLE IV**

*The physical properties of quaternary Ti-Mn-Cr-Mo alloys after a 1-hour vacuum anneal at 700° C.*

| Composition, percent<br>(balance titanium) |      |     | Ti base | Tensile properties,<br>P. S. I. |         | Percent<br>elong. |
|--------------------------------------------|------|-----|---------|---------------------------------|---------|-------------------|
| Mn                                         | Cr   | Mo  |         | Yield                           | Tensile |                   |
| 9.1                                        | 4.9  | 5.1 | Iodide  | 135,700                         | 158,400 | 10                |
| 10.1                                       | 5.2  | 5.1 | do      | 138,900                         | 144,600 | 23                |
| 8.3                                        | 5.0  | 4.7 | do      | 125,700                         | 132,700 | 19                |
| 9.2                                        | 5.1  | 5.0 | CP      | 132,300                         | 135,300 | 9                 |
| 4.4                                        | 10.0 | 4.5 | Iodide  | 124,400                         | 132,100 | 23                |
| 10.5                                       | 2.0  | 5.0 | CP      | 133,500                         | 137,900 | 13                |
| 10.5                                       | 5.0  | 2.0 | CP      | 130,700                         | 134,500 | 11                |
| 8.5                                        | 5.1  | 9.2 | Iodide  | 132,300                         | 136,600 | 20                |
| 8.6                                        | 9.8  | 4.6 | do      | 141,500                         | 150,100 | 20                |
| 4.6                                        | 5.0  | 9.3 | do      | 117,000                         | 122,700 | 17                |
| 9.2                                        | 5.0  | 5.0 | do      | 126,900                         | 128,200 | 21                |
| 9.3                                        | 7.0  | 6.7 | do      | 135,100                         | 143,000 | 24                |
| 10.4                                       | 5.0  | 5.0 | CP      | 145,200                         | 149,100 | 28                |

It will be seen that these alloys possess in general high strength combined with high ductility. That these alloys possess in general a stable beta microstructure, is shown by the bend test data of the following Table V, which gives bend test values of typical analyses as annealed and after subsequent aging for 16 hours at 400° C. and after 68 hours at 300° C.:

**TABLE V**

*Bend ductility T of samples after 1 hr. 700° C. vacuum anneal followed by heat treatment shown*

| Composition, percent<br>(balance titanium) |      |     | Ti base | As an-<br>nealed | 16 hours      | 68 hours      |
|--------------------------------------------|------|-----|---------|------------------|---------------|---------------|
| Mn                                         | Cr   | Mo  |         |                  | at 400°<br>C. | at 300°<br>C. |
| 9.2                                        | 5.0  | 5.0 | Iodide  | 0                | 0             | 0             |
| 9.2                                        | 5.1  | 5.0 | CP      | 0                | 0             | 0             |
| 10.5                                       | 5.0  | 2.0 | CP      | 0                | 0             | 0             |
| 10.5                                       | 2.0  | 5.0 | CP      | 0                | 3.2           | 1.6           |
| 8.3                                        | 5.0  | 4.7 | Iodide  | 0                | 0             | 0             |
| 8.5                                        | 5.1  | 9.2 | do      | 0                | 0             | 0             |
| 8.6                                        | 9.8  | 4.6 | do      | 0                | 3.2           | 0.8           |
| 4.6                                        | 5.0  | 9.3 | do      | 0                | 0             | 0             |
| 4.4                                        | 10.0 | 4.5 | do      | 0                | 0             | 0             |
| 9.2                                        | 5.1  | 5.0 | do      | 0                | 0             | 0             |

It will be observed that these analyses undergo no substantial change in bend ductilities as a result of these aging treatments, which indicates that there has been no rejection of a second phase.

The useful range for the ductile quaternary alloys of Tables IV and V is about 1.0 to 25% molybdenum with about 1 to 15% manganese and about 1 to 12% chromium. A preferred range for assuring optimum beta stability is about 4 to 11% manganese without 2 to 10% each of chromium and molybdenum and an aggregate content of these elements of about 17 to 23%. A particularly good alloy is one containing about 10% manganese and 5% each of chromium and molybdenum.

The alloys of the invention are preferably made by melt casting, and may optionally contain up to about 0.3% carbon, and up to 0.2% each of oxygen and nitrogen.

Depending upon the particular sample tested, unalloyed "iodide" titanium has approximately a yield strength of 27,000 p. s. i., a tensile strength of 43,000 p. s. i., an elongation of 40% and a bend ductility of 0.

Again, depending upon the sample tested, the corresponding values for unalloyed titanium of commercial purity are approximately: yield strength 51,000 p. s. i., tensile strength 76,000 p. s. i., elongation 21%, bend ductility 0.8.

It will be seen by comparison of the above values for unalloyed titanium with those of Tables I-V, inc., herein, that the tensile properties of the alloys of this invention are tremendously enhanced as compared to the unalloyed titanium, while maintaining adequate ductility for purposes of fabrication. As shown by the test data of these tables, the tensile strength of the alloys hereof ranges from a minimum of about 110,000-115,000 p. s. i. to as high as about 190,000 p. s. i. Expressed in percentages, the increase in tensile strength of the alloys herein as compared to unalloyed titanium of commercial purity, ranges from about 50% to 250%.

What is claimed is:

1. A stable and ductile alloy containing at least two elements selected from the group consisting of about 1 to 15% manganese, about 3 to 12% chromium, and about 1 to 25% molybdenum, said alloy also containing up to 0.3% carbon and up to 0.2% each of oxygen and nitrogen, balance titanium.

2. A thermally stable and ductile titanium base alloy containing about 4 to 11% manganese, about 2 to 10% each of chromium and molybdenum, up to about 0.3% carbon, up to about 0.2% each of oxygen and nitrogen, said alloy being characterized in having an ultimate strength in excess of the unalloyed titanium base metal, and in undergoing no appreciable loss of ductility on aging at temperatures up to about 400° C.

3. A stable and ductile alloy containing about 4 to 11% manganese, about 2 to 10% each of chromium and molybdenum, up to about 0.3% carbon, up to about 0.2% each of oxygen and nitrogen, and the balance titanium.

4. A thermally stable titanium base and ductile alloy containing about 4 to 11% manganese, about 2 to 10% each of chromium and molybdenum, the total content of these elements being about 17 to 23%, up to about 0.3% carbon, up to about 0.2% each of oxygen and nitrogen, said alloy being characterized in having an ultimate strength in excess of the unalloyed titanium base metal, and in undergoing no appreciable loss of ductility on aging at temperatures up to about 400° C.

5. A thermally stable and ductile alloy containing about 4 to 11% manganese, about 2 to 10% each of chromium and molybdenum, the total content of these elements being about 17 to 23%, up to about 0.3% carbon, up to about 0.2% each of oxygen and nitrogen, balance titanium.

References Cited in the file of this patent  
UNITED STATES PATENTS

2,588,007 Jaffee ----- Mar. 4, 1952  
2,596,485 Jaffee et al. ----- May 13, 1952

FOREIGN PATENTS

718,822 Germany ----- Mar. 24, 1942

OTHER REFERENCES

"Titanium," Report of Symposium December 16, 1948, sponsored by O. No. R., Dept. of the Navy, page 140.

"Product Engineering," November 1949, pages 149 and 150.

UNITED STATES PATENT OFFICE  
CERTIFICATE OF CORRECTION

Patent No. 2,829,974

April 8, 1958

Walter L. Finlay et al.

It is hereby certified that error appears in the printed specification of the above numbered patent requiring correction and that the said Letters Patent should read as corrected below.

Column 3, line 55, for "without 2 to 10%" read -- with about 2 to 10% --.

Signed and sealed this 27th day of May 1958.

(SEAL)

Attest:

KARL H. AXLINE

Attesting Officer

ROBERT C. WATSON  
Commissioner of Patents